

## UNITED STATES PATENT OFFICE.

HAROLD I. HUEY, OF SAYLESVILLE, RHODE ISLAND, ASSIGNOR TO SAYLES FINISHING PLANTS, INC., OF SAYLESVILLE, RHODE ISLAND, A CORPORATION OF RHODE ISLAND.

## PROCESS FOR PRODUCING WOOLLIKE EFFECTS ON COTTON FABRICS.

No Drawing. Application filed May 5, 1922, Serial No. 558,763. Renewed September 30, 1924.

This invention relates to processes for treating unmercerized cotton fabrics for the production of a wool-like finish.

It is now well known that if a cotton fabric be subjected to the action of concentrated sulphuric acid, a permanent structural change takes place in the fibres which remains even though the treated fabric be washed. In 1844 Mercer suggested that a cotton fabric will assume a parchment-like quality provided the sulphuric acid be of a concentration between 49.5° and 53.5° Baumé, and since that time Blondell and others have found that the change in the cellular structure of cotton goods varies as the concentration of the sulphuric acid is raised or lowered. Other factors further influence the effects produced on cotton fabrics by the acid treatment, such, for instance, as the character or condition of the fabric at the time of the acid treatment, the temperature and length of time the acid treatment continues.

It has been observed, heretofore, that the action of sulphuric acid of a concentration of less than 51° Bé., is much more intensive and imparts to cotton fabrics new properties or characteristics if the cotton has been previously mercerized and thereby rendered more susceptible to the action of the acid, and that the mercerizing luster disappears while the fabric assumes a fine, light, or wool-like nature. Repeated treatments of the mercerized fabric by sulphuric acid of 49° to 50½° Bé. concentration and alkali lye have been heretofore suggested as increasing the wool-like effects produced, provided that a treatment with one of the reagents takes place between two treatments with the other. It has been suggested, also, that transparent effects different from the mercerization effects, may be imparted to cotton fabrics by treatment with caustic alkali lye of at least 15° Baumé specific gravity at a temperature below 0° C.

The present invention, however, differs from all of these, and is based on the observation that an unmercerized cotton fabric treated with sulphuric acid of a concentration of from 51° to 53° Bé. at a temperature of about 15° C., and then with caustic soda of about one-half the strength usually employed in a mercerizing, or from 15° to 22°

Bé., takes a fine, sheer finish, and wool-like appearance. The acid treatment at the concentration and temperature indicated should not continue more than about two minutes, and preferably less, while the caustic soda treatment at the concentration indicated may continue from twenty to thirty minutes or more.

In accordance with the present invention, the cotton fabric which has not been previously mercerized is freed from the sizing, finishing agents, natural gums, and waxes by boiling, and the fabrics may be then bleached and dried.

The unmercerized fabric is then treated with sulphuric acid of a concentration between 51° and 53° Bé. at a temperature between 14° and 16° C. This treatment has a swelling action on the fabric and fulls and shrinks it. The length of time during which the action of the acid continues may vary, but preferably is less than two minutes, which is found to be sufficient to produce the desired effect.

The treated fabric is now washed and dried, after which it is subjected to the action of caustic soda at a concentration of about one-half the strength usually employed in the mercerization process or of a concentration of from 15° to 22° Bé. at a temperature of between 30° and 35° C. The strength of the caustic soda is such that it would have no mercerizing effect on fabrics not previously treated, and under the conditions and in accordance with the present invention it serves to impart to the fabric the desired sheerness, firmness, and finished wool-like appearance.

The treatment with the caustic soda at the concentration described may continue for about one half hour, at the end of which time the fabric is washed and dried. During the process the fabric preferably remains unstretched and no tension is placed upon it that would tend to eliminate the desired crepe-like effect.

## What is claimed is:

1. The process described for imparting to unmercerized cotton fabrics a wool-like appearance, consisting in causing concentrated sulphuric acid of 51° to 53° Bé. to act upon the fabric, washing and drying the fabric and then subjecting the fabric to the action

of caustic soda of concentration of from 15° to 22° Bé. at a temperature between 30° and 35° C. and washing the treated fabric.

2. The process described for imparting to 5 unmercerized cotton fabrics a wool-like appearance, consisting in causing concentrated sulphuric acid of from 51° to 53° Bé. to act upon the unmercerized fabric at a temperature of from 14° to 16° C. then washing and 10 drying the fabric, subjecting the fabric to the action of caustic soda of a concentration between 15° and 22° Bé., and washing the treated fabric.

3. The process described for imparting a 15 wool-like appearance to unmercerized cotton fabrics, consisting in boiling the unmercerized fabric and drying it, then causing sulphuric acid of concentration from 51° to 53° Bé. to act upon the fabric for not more than 20 two minutes, then washing and drying the

fabric and then subjecting the fabric to the action of caustic soda of a concentration of between 15° to 22° Bé. at a temperature above 30° C., and then washing the fabric.

4. The process described for imparting to 25 unmercerized cotton fabrics a wool-like character, both as to feel and appearance, consisting in first eliminating the natural gums, waxes, and finishing agents from the unmercerized fabric, then bleaching the fabric, then causing sulphuric acid of concentration between 51° and 53° Bé. to act upon the fabric at a temperature of from 14° to 16° C., washing and drying the fabric, then subjecting the fabric to the action of caustic soda of from 15° to 22° Bé., and then washing the fabric.

In testimony whereof, I have signed my name to this specification.

HAROLD I. HUEY.